

March 24, 1936.

H. T. BEBB  
CONTINUOUS ENAMELWARE MANUFACTURE

2,035,363

Filed Oct. 12, 1932

3 Sheets-Sheet 1



Fig. 2

Inventor  
H. T. Bebb

By *Grease and Bishop* Attorneys

March 24, 1936.

H. T. BEBB

2,035,363

CONTINUOUS ENAMELWARE MANUFACTURE

Filed Oct. 12, 1932

3 Sheets-Sheet 2



Fig. 5

Inventor

*H.T. Bebb*

By *Grease and Bishop*  
Attorneys

March 24, 1936.

H. T. BEBB

2,035,363

## CONTINUOUS ENAMELWARE MANUFACTURE

Filed Oct. 12, 1932

3 Sheets-Sheet 3



Fig. A

Inventor

*H.T.Bebb*

३३४

Grease and Bishop

Autumnus

## UNITED STATES PATENT OFFICE

2,035,363

CONTINUOUS ENAMELWARE  
MANUFACTURE

Harry T. Bebb, Canton, Ohio, assignor to The  
Canton Stamping & Enameling Company,  
Canton, Ohio, a corporation of Ohio

Application October 12, 1932, Serial No. 637,440

17 Claims.

(Cl. 91—73)

My invention relates to the continuous manufacture of vitreous enamel ware, and more particularly to an improved method of making mottled gray ware with a single coat of vitreous enamel; as, for instance, cooking or kitchen utensils made of sheet steel coated with a vitreous enamel to protect the metal from rusting and from the action of acids in use.

In the manufacture of such enamel ware, a liquid enamel coating is first applied to the ware, usually by dipping, and the dipped ware is then dried; and to obtain a uniform mottled effect, it has been discovered that the drying must be done by exposing the free surface of individual pieces to the atmosphere, under controlled conditions of different relative movements, temperatures and humidities in substantially immediate successive periods of time during which the drying is being effected, to form and merge together the comparatively small rust spots or blotches of different colors or shades, which are required for producing the desired appearance.

In the usual method of making such ware, the dipped pieces have been placed on stationary racks located in a drying room, through which heated air has been moved; and after the ware was sufficiently dried, it was then burned in a furnace, which requires a manual transfer from drying rack frames to burning rack frames, for which as many as seven men were sometimes employed in actual practice.

The problem of making uniformly mottled enamel ware products has been difficult to solve, no doubt, because even though sheet metal of the proper grain structure, analysis and cleanliness is coated with a liquid vitreous enamel of the proper composition and consistency, the mottled effect is obtained by a rusting or oxidation in spots or portions of the surface of the metal by certain ingredients or moisture of the enamel coating; and a control of the size and a merging of the spots can only be obtained by peculiar and exact drying operations under certain conditions of time, and of the movement, the temperature, and the humidity of the atmosphere to which the ware, with the enamel coating thereon, is exposed during successive drying periods.

For the purpose of obtaining the best results in making enamel ware, it is preferred to select pickled and annealed rolled iron or steel sheets, which may be of from 24 to 30 gauge, known to the trade as P & A Enamel Stock, having a uniform average size of grain structure, and having a composition or analysis and ductility which permits a deep drawing of the sheet metal.

The enamel stock is first stamped or drawn into the desired shape for a cooking utensil or other article, from which all grease and surface dirt is removed by an alkali solution at a boiling temperature, and all oxidation is then removed by a sulphuric acid pickling solution at a temperature of from 140° to 180° F.; after which all trace of acid is removed by washing in clear running water, and the surface is neutralized and further oxidation avoided until the shapes are coated, by another alkali bath at a temperature of from 140° to 150° F.; which is followed by a quick drying in an oven hot enough to completely remove all moisture from the surface of the shapes, within four or five minutes; after which the same are ready for the application of a liquid vitreous enamel.

There are many liquid vitreous enamels in common use, and a well known formula may be followed, which includes a mixture of borax, 60 pounds; feldspar, 56 pounds; silica, 40 pounds; saltpeter, 3 pounds; soda ash, 20 pounds; fluor spar, 12 pounds; antimony, 3 pounds; cryolite, 10 pounds; bone ash, 6 pounds; and manganese oxide, 12 pounds; the same being smelted at about 2200° F. into molten glass, which is shattered into small fragments by being run out of the smelter into cold water, and then ground in a ball mill for some twelve hours, wherein ball clay and water are added, to form a liquid enamel coating of about the consistency of thick cream.

The cleaned, pickled, and neutralized sheet steel shapes or pieces of ware are taken from the quick drying oven by the dipping operator and individually immersed in the liquid enamel solution, wherein it is given a single coating; the piece being suitably rotated and manipulated by the operator to give it a uniform single coating or covering of a single thickness of the liquid enamel which adheres to the surface of the shape.

The liquid coating on the metal ware is then ready for drying and burning, and according to the improved method, the drying operations include a continuous series in substantially immediate succession of several more or less distinct time periods, during which the drying is effected under different conditions of movement, temperature, and humidity of the atmosphere, in and by which the drying is effected.

During the first drying period, the liquid coating on the ware may be exposed for from twenty to twenty-five minutes to the atmosphere, by slowly moving the ware in the ordinary atmosphere and air currents normally present in the drying room of an enamel ware manufacturing

plant, which may have a temperature of from 70° to 90° F., with a normal degree of humidity, depending upon the season of the year; the period of the exposure being such as to gradually 5 dry the wet enamel coating until it is fixed or set on the surface of the sheet metal, and until an oxidation resulting from the rusting of the metal by the wet coating, becomes visible in the form of small spots, more or less scattered, in some portions of the pieces of work.

10 During the second drying period, the enamel coating on the work may be exposed for some thirty-five to forty minutes in a constantly moving and actively agitated atmosphere, heated to a 15 temperature according to a dry bulb reading of from 90° to 115° F. and according to a wet bulb reading of from 65° to 85° F., at a humidity of approximately 25% to 35% of saturation, until most of the moisture is removed from the enamel 20 coating which has been set during the first period; the exposure being extended during such a period as will initiate the oxidation or rusting of small adjacent spots to form and merge together in a uniform manner throughout the 25 tire surface of each one of the coated shapes.

During the third drying period, the enamel coating on the ware may be exposed for from five to ten minutes in a moderately moving atmosphere, heated to a temperature from 140° to 30 160° F., with a normal degree of humidity; and this period may be extended until the formation and merging of comparatively small adjacent oxide or rust spots has been completed throughout the entire surface of each enamel coated shape, 35 but before the moisture has been entirely eliminated to produce a bone dry enamel coating.

And during the fourth drying period the enamel coating on the ware may be exposed for from five to ten minutes in a moderately moving atmosphere, heated to a temperature of from 160° to 40 200° F., with a normal degree of humidity; and this period is extended until the moisture in the enamel coating has been so completely eliminated as to produce a bone dry condition of the same; 45 in which condition the enamel coated ware is ready for the final step of burning.

It will be understood, however, that the third and fourth drying periods are so nearly alike, that they may be considered together as a single 50 period, during which the enamel coating may be exposed for from ten to twenty minutes in a moderately moving atmosphere, heated to a temperature of from 140° to 200° F., with a normal degree of humidity; and such period is extended 55 until the formation and merging of comparatively small adjacent rust spots has been completed throughout each enamel coated shape, and the moisture in the enamel coating has been so completely eliminated as to produce a bone dry condition of the same.

And it will be understood that the several conditions and degrees described for the substantially immediate successive periods of drying may be modified from the ranges which have been 60 enumerated, depending upon different atmospheric conditions during the various seasons, and upon variations in the details of the composition of the liquid enamel coating, and more particularly, upon variations in the degree of one feature 65 with respect to another, during the several drying periods; the described conditions being illustrative of those conditions which an extended experience in the actual use of the improved method, has resulted in the very successful production 70

75 of single coated uniformly mottled enamel ware, as described.

In the final step of burning, the enamel coated ware may be exposed during a period of from ten to twelve minutes, beginning and ending with an 5 initial and final temperature of some 700° F., for about four minutes each, and including an intervening maximum temperature of from 1200° to 1640° F. for about four minutes; the period of the 10 burning exposure being extended until the enamel coating which has been completely dried, is completely vitrified on the metal base or body of the ware; and because of the described manner in which the enamel coating has been dried, the 15 vitrified coating presents a substantially uniform mottled appearance of closely adjacent small spots merged together.

During the drying and burning periods thus described, the enamel coated shapes may be continuously carried from the drying room through 20 a series of successive drying zones or chambers and a burning furnace, and back into the drying room for cooling, by being individually mounted by the dipping operator upon racks depending from a continuously operating endless chain conveyor.

The continuous method thus described may be carried out by the apparatus which is disclosed in my copending application filed January 22, 1931, Serial No. 510,447, matured in Letters Patent No. 1,890,897, for Continuous enamel ware apparatus; the present application being a continuation in part of the common subject matter disclosed in that application, which is a copending continuation in part of the common subject matter disclosed in my earlier application filed May 13, 1929, Serial No. 362,834, for Continuous enamel ware manufacture; and such apparatus is illustrated in the accompanying drawings forming part hereof, in which—

40 Figure 1 is a diagrammatic plan view of the apparatus;

Fig. 2, an enlarged fragmentary diagrammatic transverse sectional view thereof, as on line 2—2, 45 Figs. 1 and 3;

Fig. 3, an enlarged fragmentary longitudinal sectional view thereof, as on line 3—3, Figs. 1 and 2; and

Fig. 4, a diagrammatic outline plan of the apparatus.

Similar numerals refer to similar parts throughout the drawings.

The apparatus may include a dryer 10 and a furnace 11 which are preferably located in a zone 12, which may be located in an enclosed room, such as the ordinary drying room of an enamel 55 ware manufacturing plant.

A dryer 10 is preferably built of refractory walls 13 which may form a plurality of successive communicating zones or chambers 14, 15 and 16; 60 and the first zone or chamber 14 of the dryer, communicates with the zone 12 in which the dryer as a whole is located, as by means of an inlet passageway 17 formed in the dryer walls.

For conserving space, the drying chambers 65 14, 15 and 16 are preferably located side by side, the chambers 14 and 15 having a common partition wall 18, and the chambers 15 and 16 having a common partition wall 19; with communicating openings 20 and 21 in the respective walls 70 at opposite ends of the dryer, between the adjacent chambers.

The inlet passageway 17, as illustrated, is preferably provided at one end corner of the dryer 10; and at the delivery end of chamber 16 may 75

be provided an end closure wall 22 having formed therein an outlet opening 23 for the dryer.

This outlet opening 23 may communicate with the zone 12, as illustrated, and one end wall of the burning furnace 11 may be located directly opposite the end wall 23 of the chamber 16; and the furnace wall 24 has formed therein an inlet opening 25 opposite the outlet opening 23 of the dryer, and the furnace wall 24 has also formed therein an outlet opening 26 laterally spaced from the opening 25; or, if desired, the dryer may communicate directly with the furnace.

A continuous endless chain conveyer 27, or the like, passes through the inlet passageway 17 into the dryer and through the successive chambers thereof, thence through the dryer outlet opening 23, and through the furnace inlet opening 25 into the interior 28 of the furnace and thence out of the furnace outlet opening 26 into the zone 12, and thence back to the dryer.

As illustrated, the first drying chamber 14 has a greater volume than the successive drying chambers, for accommodating therein substantially 4 times the length of chain conveyer as is accommodated in the chamber 15, and the chamber 16 has a volume less than the volume of the chamber 15 for accommodating less length of the chain conveyer; and the entire length of the dryer may be approximately one hundred and fifty feet, for the purposes of the present invention.

Accordingly, with a constant speed of travel of the chain conveyer 27, which speed may be from 14 ft. to 20 ft. per minute, the enamel coated shapes indicated generally by 29 and carried by the conveyer, as by means of racks 30 depending from the conveyer 27, are subject for different periods of time to the successive atmospheres of the successive zones or chambers.

Means are provided for maintaining the substantially immediate successive zones or chambers of the apparatus at different temperatures, for maintaining differently directed blasts of air in each drying chamber and for maintaining different humidities in each drying chamber.

The temperature of the zone 12 as aforesaid may be the temperature of the ordinary drying room of an enamel ware manufacturing plant, and may be from 70° to 90° F. The temperature of the drying chamber or zone 14 is preferably maintained for the purposes of the present invention, at 65° to 85° F. wet bulb reading, and at 90° to 115° F. dry bulb reading, with a humidity of from 25% to 35% of saturation. The temperature of the drying chamber or zone 15 is maintained at from 140° to 160° F., and the temperature of the drying chamber or zone 16 is maintained at from 160° to 200° F.

The interior of the furnace 28 may be maintained at its end adjacent the inlet opening 25 and the outlet opening 26, at substantially 700° F., and at the other burner end of the furnace, the temperature is preferably from 1200° to 1640° F.

While the heating means and the air moving means for the drying chambers may be separate, in the embodiment illustrated in the drawings, common heating and air blasting means are provided by blowing or blasting hot air through the several chambers.

All the chambers of the dryer 10 may have a common bottom wall 31 which is likewise the top wall of an exhaust chamber 32. The wall 31 has a plurality of openings 33 formed therein for

each of the chambers 14, 15 and 16 for providing a communication between each drying chamber and the exhaust chamber 32.

Vertically directed blasts of hot air are supplied to the drying chamber 14 as by means of a blower 34 whose inlet duct 35 is connected with a source of hot air, and whose outlet duct 36 communicates with the top of the chamber 14 through a plurality of branch outlet ducts 37.

The chambers or zones 15 and 16 are maintained at their differential temperatures and provided with vertical blasts of air as by means of a blower 34' whose inlet duct 35' is connected with a source of air hotter than the source for the blower 34, and whose outlet duct 36' communicates with the upper portions of the chambers 15 and 16 through branch ducts 37'a and 37'b, respectively, the ducts 37'b having the greater capacity.

One or more booster or exhaust fans 38 may be located in the exhaust chamber 32 for facilitating drawing the differentially heated air vertically through the several drying chambers 14, 15 and 16; and a plurality of horizontally directed fans 43 may be located in the several drying chambers 25 near the bottom thereof for moving differently directed blasts of air therein; and/or a plurality of downwardly inclined directed fans 40' may be located near the top of the several drying chambers, at one end thereof, for blowing air currents downward toward the other end thereof, and into the open upper side of the several pieces of ware.

The humidity of the several drying chambers is separately controlled both by the relative volumes of the chambers, and by the use of a supply of water, which may be contained in pans 41 located in the chamber 14; or the humidity of the atmosphere may be increased or decreased by the use, or non-use, of steam sprays 42 from an apertured steam pipe 42', as shown in the upper middle portion of the more humid chamber 14.

It will be understood that some of the walls of the several drying chambers may have doors or shutters therein or may be entirely open at one end, as indicated at 43 and 44 in Fig. 4, for the more humid chamber 14; because such openings may be desirable for supplying a greater volume of the moving atmosphere which is highly heated and humidified for the purpose of the second period of drying carried on in the particular chamber.

The different periods of drying are provided, because of the precise conditions of time, temperature and humidity, which are required for initiating a uniformly mottled rusting of the metal by the wet coating; and although the first period of drying may proceed in ordinary atmospheric conditions until scattering rust spots are visible, a further drying under the same conditions results in the formation of relatively large rust spots, blotches or streaks, which are not only unsightly, but the rust penetrates so deeply into the metal as to form depressed spots or streaks when the ware is burned.

For that reason, the drying during the second period is retarded, by increasing the humidity of the atmosphere, and at the same time a uniformly mottled rust is facilitated, by increasing the temperature of the atmosphere; so that the mottled rusting is initiated throughout the entire surface of each shape, as well as throughout the entire surface of the many different sizes of shapes which may be continuously and contem-

poraneously dried and burned by the present method.

In other words, there must be a change in and a coordination between the time, the temperature and the humidity, after small scattering rust spots begin to form, until adjacent small rust spots are formed and merge throughout the entire surface of each shape, as well as of many different sizes and kinds of shapes, which may 10 include various kitchen utensils, from small cups, stew pans and coffee pots, to very large dish pans and the like.

There must also be a substantially continuous and substantially immediate succession of the several drying periods, and preferably of the 15 burning period; because an exposure to the ordinary atmosphere for any considerable length of time between the first and second drying periods, will result in an excessive and a non-uniform 20 oxidation or rusting; and an exposure to the ordinary atmosphere between the second and third, and the third and fourth drying periods, for any considerable length of time, will also result in an excessive oxidation and a non-uniform completion 25 of the mottled rusting which has been initiated during the second period.

And likewise, if the bone dry enamel coating at the completion of the drying operations is exposed to the ordinary atmosphere for any considerable length of time, it will absorb moisture therefrom, which will cause a further and an excessive oxidation, and destroy the uniform mottled rusting which has been effected, as described, and which can only be preserved by promptly 35 burning the ware, for accomplishing the purposes of the present invention.

And finally, the continuous movement of the ware, from the time it is dipped and placed upon the endless conveyer racks, until it has been 40 dried and burned to produce the finished product as described, and until the same has been cooled and removed to ware trucks; avoids the loss of marred ware, which always results from a manual handling of the individual shapes to and from 45 carrying boards, trays, trucks and the like, in common practice.

Such a marring causes a loss of defective ware, which may amount to from 10% to 15% of the entire production; and it is difficult, if not impossible, to avoid the same, because the smooth, 50 wet enamel coating is so delicate that it is impaired and defaced by the slightest touch of the hand of an operator, or a contact with an adjacent piece of ware or other object; and the bone dry coating is merely a thin film of the powdered enamel, which is likewise disfigured and damaged, if not entirely removed, by the touch or contact of a hand or another object.

In addition to the saving of loss from damaged 60 ware, the continuous movement of the enameled shapes upon an endless conveyer, in substantially immediate succession throughout the drying and burning periods, saves the time and expense of the labor which would otherwise be required for 65 handling the ware during these operations; and because the dipping, burning, drying, cooling and removing operations are all continuously coordinated and completed within an hour and a half, there is no loss of labor or delay in production, 70 which frequently occurs when one or more of the several periods of manufacture are independently or separately carried on, as in common practice.

I claim:—

1. The method of making mottled enamel ware, 75 which consists in drying a wet enamel coating

upon a sheet steel shape by exposing the same in an ordinary atmosphere at a temperature of from 70° to 90° F., for from 20 to 25 minutes; then exposing the same in an actively moving atmosphere at from 65° to 85° F. wet bulb reading and from 90° to 115° F. dry bulb reading, that is with a humidity of from 25% to 35% of saturation, for from 35 to 40 minutes; then exposing the same to a moderately moving atmosphere at from 140° to 160° F., for from 5 to 10 minutes; then exposing the same in an atmosphere at from 160° to 200° F., for from 5 to 10 minutes; and then burning the enamel coated shape. 5

2. The method of making mottled enamel ware, 15 which includes drying single wet enamel coatings upon sheet steel shapes by exposing the same in an ordinary atmosphere until small scattered rust spots are visible, then promptly exposing the same in a heated humid moving atmosphere 20 until the forming and merging of small adjacent rust spots is initiated throughout the surfaces of the shapes, then promptly exposing the same in a higher heated moving atmosphere until the forming and merging of the rust spots is completed, then promptly exposing the same to a higher heated atmosphere until the enamel coating is bone dry, and then promptly exposing the ware to a burning atmosphere, all while moving the shapes continuously through each and all of 30 the atmospheres. 25

3. The method of making mottled enamel ware, which includes drying a wet enamel coating upon a sheet steel shape by exposing the same in an ordinary atmosphere until small scattered rust 35 spots are visible, then exposing the same in a heated humid moving atmosphere until the forming and merging of small adjacent rust spots is initiated throughout the surface of the shape, then exposing the same in a higher heated moving atmosphere until the forming and merging of the rust spots is completed, then exposing the same to a higher heated atmosphere until the enamel coating is bone dry, and then burning the 40 enamel coated shape. 45

4. The method of making mottled enamel ware, which includes drying a wet enamel coating upon a sheet steel shape by exposing the same in an ordinary atmosphere until small scattered rust 50 spots are visible, then exposing the same in a heated humid moving atmosphere until the forming and merging of small adjacent rust spots is initiated throughout the surface of the shape, then exposing the same in a higher heated moving atmosphere until the forming and merging 55 of the rust spots is completed, and then exposing the same to a higher heated atmosphere until the enamel coating is bone dry.

5. The method of making mottled enamel ware, which includes drying a wet enamel coating upon 60 a sheet steel shape, by exposing the same in an ordinary atmosphere until small scattered rust spots are visible, then exposing the same in a heated humid moving atmosphere until the forming and merging of small adjacent rust spots is 65 initiated throughout the surface of the shape, and then exposing the same to a higher heated atmosphere until the forming and merging of the rust spots is completed and the enamel coating is bone dry. 70

6. The method of making mottled enamel ware, which includes the steps of drying a wet enamel coating upon a sheet steel shape by exposing the same in a heated humid moving atmosphere until the forming and merging of small adjacent 75

rust spots is initiated throughout the surface of the shape, and then exposing the same to a higher heated moving atmosphere until the forming and merging of the rust spots is completed and the enamel coating is bone dry.

5 7. The method of making mottled enamel ware, which includes the steps of drying a wet enamel coating upon a sheet steel shape, by exposing the same in an ordinary atmosphere until small scattered rust spots are visible, and then exposing the same in a heated humid moving atmosphere until the forming and merging of small adjacent rust spots is initiated throughout the surface of the shape.

10 8. The method of making mottled enamel ware which includes the step of drying a wet enamel coating by exposing the same in an actively moving atmosphere at from 60° to 85° F. wet bulb reading, and from 90° to 115° F. dry bulb reading, that is, with a humidity of from 25% to 35% of 15 saturation, for from 35 to 40 minutes.

15 9. The method of making enamel sheet steel ware and the like, which includes continuously moving and subjecting such ware having liquid enamel applied thereon to immediately successive 20 drying atmospheres, beginning with the ordinary temperature of a drying room and each successive atmosphere being independently maintained at substantially higher drying temperature than the 25 previous atmosphere to uniformly form and then merge comparatively small adjacent rust spots throughout the surface of the ware, and then burning the ware.

20 10. The method of making enamel sheet steel 30 ware and the like, which includes continuously moving and subjecting such ware having liquid enamel applied thereon to ordinary atmospheric conditions for a substantial length of time and then to immediately successive drying atmospheres, each drying atmosphere acting on the 35 ware for a substantial length of time, and each atmosphere being independently maintained at a substantially higher drying temperature than the previous atmosphere to uniformly form and then merge comparatively small adjacent rust spots 40 throughout the surface of the ware.

45 11. The method of making enamel sheet steel ware and the like, which includes continuously moving and drying such ware having liquid 50 enamel applied thereon, by subjecting the ware in immediate succession to blasts of heated air, beginning with the ordinary temperature of a drying room and each successive blast being maintained at a substantially higher temperature than a previous blast.

55 12. The method of making enamel sheet steel ware and the like, which includes continuously

moving and subjecting such ware having liquid enamel applied thereon to immediately successive drying atmospheres, beginning with the ordinary temperature of a drying room and each successive atmosphere being independently maintained at a higher drying temperature with a different degree of humidity, than the previous atmosphere.

5 13. The method of making enamel sheet steel ware and the like, which includes continuously moving and subjecting such ware having liquid enamel applied thereon to ordinary atmospheric conditions for a substantial length of time, and then to immediately successive drying atmospheres, each atmosphere acting on the ware for a substantial length of time and each atmosphere being independently maintained at a higher temperature with a different degree of humidity than the previous atmosphere.

10 14. The method of making enamel sheet steel 15 ware and the like, which includes continuously moving and drying such ware having liquid enamel applied thereto, and subjecting the ware in immediate succession to differently directed blasts of heated air, beginning with the ordinary 20 temperature of a drying room and each successive blast being maintained at substantially higher 25 drying temperatures than a previous blast.

25 15. The method of making enamel sheet steel 30 ware and the like, which includes continuously moving and drying liquid enamel on such ware by subjecting the ware in immediate succession to blasts of air, beginning with the ordinary temperature of a drying room and each successive 35 blast being maintained at a substantially higher drying temperature with a different degree of humidity than a previous blast.

30 16. The method of making enamel sheet steel 40 ware and the like, which includes continuously moving and drying a wet enamel coating on such ware in a normal atmosphere until scattered rust spots appear, then facilitating the forming and merging of rust spots while retarding the drying in a higher than normal drying heat and degree of humidity, and then completely drying the coating in a still higher atmospheric heat.

45 17. The method of making enamel sheet steel 50 ware and the like, which includes continuously moving and drying a wet enamel coating thereon in normal atmosphere until scattered rust spots 55 appear therein, then facilitating the forming and merging of rust spots while retarding the drying in a higher than normal drying heat and degree of humidity, and then completely drying the coating in a still higher atmospheric heat and a normal degree of humidity.

HARRY T. BEBB.